

Sept. 11, 1956

J. M. CRANMER

2,762,758

## ASPHALT MANUFACTURE

Filed May 5, 1953



INVENTOR.  
JOHN M. CRANMER  
BY Robert D. Slynn  
AGENT

# United States Patent Office

2,762,758

Patented Sept. 11, 1956

1

2,762,758

## ASPHALT MANUFACTURE

John M. Crammer, Riverside, R. I., assignor to Socony  
Mobil Oil Company, Inc., a corporation of New York

Application May 5, 1953, Serial No. 353,153

4 Claims. (Cl. 196—74)

This invention has to do with a process for manufacturing asphalt and, more specifically, has to do with improvements in the manufacture of air blown asphalt.

As is well known in the art, air blown asphalts have been prepared by air-oxidizing various petroleum residues and/or fractions in heated stills or towers and the like. Difficulties incident to air blowing of an asphalt charge stock, have been control of asphalt charge and air and control of the resultant oxidation temperature. In general, it has been necessary to reduce the flow of asphalt charge and/or the air charge in order to prevent the temperature from rising excessively. Obviously, a reduced flow rate is responsible for a curtailing or slowing up of production in a given operating unit. In addition, failure to control one or both of the foregoing factors has led to the formation of explosive mixtures.

Numerous techniques have been resorted to in an effort to provide better control over the air-blowing operation. For example, steam and/or air have been introduced into a heated asphalt charge stock to provide better agitation of the heated asphalt charge stock, and cooling of the latter can be effected by circulating a suitable cooling medium through a coil disposed in the reaction vessel; these techniques are described by E. W. Gard and P. Subkow in United States Letters Patent 1,911,114. Cooling by means of an inside coil is subject to several short-comings. For example, the amount of cooling which can be realized is limited by the amount of heat exchange surface so installed. Moreover, the outer surface of the coil becomes coated with carbon and other materials, with the result that heat exchange efficiency decreases. Additionally, the still or unit must be cleaned periodically to remove coke and other materials, and the coil interferes with the cleaning operation, thereby making the latter more expensive.

A later development involves the introduction of steam into the vapor space of the reaction vessel, in order to dilute the vapors therein and thereby to prevent the formation of an explosive mixture. The latter development is described by S. Tijmstra in 1,975,563. Although steam is effective as a diluent, it is necessary to use excessive quantities of the same in order to cool the vapor space, and, even though large quantities of steam are so used, little or no cooling of the reaction mixture is accomplished.

Another procedure considered for controlling the oxidation temperature is explained by B. G. Aldridge in 1,988,766. The procedure of the last-mentioned patent calls for injection into the heated asphalt charge stock of a volatile liquid such as water; water serves as a cooling medium. This procedure is characterized by several disadvantages. It is necessary to exercise considerable operating care and to use controls in order to prevent asphalt from flowing back into the water inlet line. When asphalt backs up into the water line, it is cooled and deposits in the line such that water can not come through the line and flow into the unit to serve the intended purpose. Another disadvantage in the Aldridge procedure is

2

the need for close control over the quantity of water so added; when an excessive quantity of water is introduced into a hot asphalt charge, the water is converted into a large volume of steam with the result, that the asphalt charge surges up through and out of the still.

Although steam has been introduced hitherto into the vapor space of a reaction vessel above the heated asphalt charge stock, as described by Tijmstra, and although water has been injected directly into the heated asphalt charge stock, as described by Aldridge, it has been generally recognized in the industry that water—as opposed to steam—should not be allowed to come in direct contact with hot asphalt. In the past, water has been introduced by accident into a heated asphalt charge, with disastrous results. Water coming into contact with the heated charge, at 300—500° F., so disturbs the equilibrium that the charge surges to the top of the vessel and overflows. In some instances, in fact, the surge has been so pronounced that the top of the vessel has been ruptured and destroyed.

Despite the apprehensions of those working in this industry, it has now been established that water can be used safely and satisfactorily as a coolant when introduced into the vapor space of the reaction vessel and on to the surface of the asphalt charge being air blown in the manner described below.

It is an object of this invention, therefore, to provide a process for manufacturing asphalt with close control over the temperature within the reaction vessel. It is also an object of this invention to provide a process characterized by a high degree of safety in operation. Another object is to provide a process characterized by complete flexibility in the amount of cooling required and by efficient heat exchange. Still another object is the provision of a process of low installation, operating and maintenance expenses. Other objects of the invention will be apparent from the following description.

It has now been found that the foregoing objects are accomplished by introducing a controlled amount of water into the vapor space of the reaction vessel and onto the liquid surface of the heated asphalt charge stock being air blown. The heated asphalt charge is maintained at a sufficiently high temperature when the water is so introduced, such that the water is completely evaporated when it comes into contact with the surface of the asphalt charge. In practice, the blowing temperature is maintained sufficiently above the boiling point of water to insure complete vaporization of the added water.

As illustrated in the attached drawing, a suitable asphalt charge stock at about 425° F. in valved line 1 is introduced into a lower section of still 2. Air is added to the still through line 3, and is dispersed into the asphalt charge stock through air nozzle pipe, turbo aerator or spider 4. The liquid level of the asphalt charge stock is indicated by 5. By way of illustration about 800 cubic feet per minute of air and 80—90 gallons per minute of a Kuwait (Near East) flux having a softening point of 80—85° F., are so added to still 2. The temperature of the still is maintained at about 500° F.

The temperature in still 2 is readily controlled by introducing a controlled quantity of water through line 6 into the vapor space of still 2. It will be understood that one or more lines such as 6 can be used, that a spray or battery of sprays can be used to bring water into the still, and that meters and coolers can be included in line 6; all are well-known expedients in the art. The quantity of water so added to the still can be related to the temperature within the still by such means, more water being added as the temperature is increased and less water being added as the temperature is decreased. With the quantities of charge stock and air given above, 0.5—4 gallons of water are added during a period of one minute.

As shown, the outlet of water line 6 is above the asphalt level 5. Line 6 is generally at least several feet above the asphalt level, as for example, in a unit sixty feet high and with the asphalt level (5) at about the forty-two foot mark.

With the aforementioned addition of water, the temperature of the still is maintained within a range of  $\pm 1^{\circ}$  F. In contrast to this, when water was omitted from the procedure, temperature control was unsatisfactory. In addition, it was necessary—when water was absent—to resort to such expedients as restricting the air flow and/or the asphalt charge in order to control the temperature.

Gases in still 2 are removed through line 7. The gases are principally nitrogen, a small amount of oxygen, water vapor formed in the oxidation reaction and steam from the added cooling water, and oil vapors. The asphalt in still 2 generally comprises about seventy per cent of this vessel, allowing for a vapor space of about thirty per cent. Asphalt is withdrawn from still 2 through either or both of valved lines 8 and 9 and is finally removed through line 10.

Although the temperature of operation is shown above to be about 500° F., it is to be understood that any temperatures suitable for an asphalt blowing operation can be used in the procedure described herein. Generally, however, preferred operating temperatures fall within the range of 450-550° F. when no catalyst is used. Temperatures as low as about 350° F. is used when a suitable catalyst is employed.

It is also contemplated herein that catalysts or modifying materials can be used in the preparation of asphalts. For example, phosphoric acid can be added to the asphalt charge stock, either to line 1 or a separate line (not shown) with an inlet positioned above or below the asphalt level 5, in which event the operating conditions are preferably those described in copending application Serial No. 277,631, filed March 20, 1952.

Air is used as the source of oxygen in view of its low cost and availability.

The operating technique of this invention is also useful for contacting oxidizing gases with other oils such as animal, marine, mineral and vegetable oils. By way of illustration, rapeseed oil can be effectively air-blown to a bodied oil useful in compounded lubricants.

It is to be understood that the operating technique described herein is applicable to batch operation and to continuous operation.

In a continuous operation, it has been found that 2000 barrels per day of a 130° F. melting point asphalt can be produced in a given unit with no cooling water added. In contrast, using the same unit and the same charge stock under comparable operating conditions, but with four gallons of water per minute added in accordance with the new technique, 3,000 barrels per day of the same asphalt product have been produced. This is an increase of fifty per cent in the capacity of a single operating unit.

The asphalt charge stocks suitable for use herein can be of varied character. Broadly, any petroleum residuum or flux, remaining following separation therefrom of vaporizable hydrocarbons through lubricating oil fractions, or any relatively high molecular weight extract obtained by petroleum refining, can be used. For example, residua from Pennsylvania, Mid-Continent, California, Middle-East, Near-East, Venezuela, etc. crudes can be used. Or in other words, residua from paraffinic, naphthenic, aromatic, high sulfur, etc. stocks are suitable. It will be recognized, of course, that differences in charge stocks are reflected in differences in the character of the final products contemplated herein, and such differences are indicated below. Typical advantageous charge stocks are a Casper flux having an 85-90° F. softening point, which is representative of a Mid-Continent charge; Lagunillas fluxes having softening points of 70° F. and 120° F., such materials typifying Venezuelan residua charges; a 27% Kuwait residuum having an 80-85° F. softening point, and a 24% Kuwait residuum having a 90° F. softening point, such typifying Near-East charges; a tar having a 95° F. softening point and obtained by a Duo-Sol treat of a heavy lubricating oil, and a tar having a 125° F. softening point and obtained by a Duo-Sol treat of a heavy lubricating oil.

I claim:

1. In the manufacture of asphalt wherein an asphalt charge stock is air blown at an elevated temperature in a vessel in which a vapor space is maintained above the liquid level of the asphalt charge stock being air blown therein, the improvement which comprises: introducing into the said vapor space and onto the heated asphalt charge stock, liquid water in an amount sufficient to control the temperature of said asphalt charge stock, and insufficient to so disturb the equilibrium that the asphalt charge surges to the top of the vessel and overflows said asphalt charge stock being maintained at a temperature above the boiling point of water.

2. In the manufacture of asphalt wherein an asphalt charge stock is air blown at a température between about

350° F. and about 550° F., in a vessel in which a vapor

space is maintained above the liquid level of the asphalt

charge stock being air blown therein, the improvement

25 which comprises: introducing into the said vapor space

and onto the heated asphalt charge stock, liquid water in

an amount sufficient to control the temperature of said

asphalt charge stock, and insufficient to so disturb the

equilibrium that the asphalt charge surges to the top of

30 the vessel and overflows said asphalt charge stock being

maintained at a temperature above the boiling point of

water.

3. In the manufacture of asphalt wherein an asphalt

charge stock is air blown at a temperature of about 500°

35 F., in a vessel in which a vapor space is maintained above

the liquid level of the asphalt charge stock being air

blown therein, the improvement which comprises: intro-

35 ducing into the said vapor space and onto the heated

asphalt charge stock, liquid water in an amount sufficient

40 to control the temperature of said asphalt charge stock,

and insufficient to so disturb the equilibrium that the

asphalt charge surges to the top of the vessel and over-

flows, said asphalt charge stock being maintained at a

45 temperature of about 500° F., the said asphalt being

charged to the vessel at the rate of about 80 to 90 gallons

per minute, the air being charged at the rate of about

800 cubic feet per minute and the water being charged

45 to the vessel at the rate of about 0.5 to 4 gallons per

minute.

4. In the manufacture of asphalt wherein an asphalt

charge stock is air blown at a temperature of about 500°

50 F., in a vessel in which a vapor space is maintained above

the liquid level of the asphalt charge stock being air

blown therein, the improvement which comprises: intro-

55 ducing into the said vapor space and onto the heated

asphalt charge stock, liquid water in an amount sufficient

to control the temperature of said asphalt charge stock,

and insufficient to so disturb the equilibrium that the

asphalt charge surges to the top of the vessel and over-

60 flows, said asphalt charge stock being maintained at a

temperature of about 500° F., the ratio between the

rates of asphalt charge stock, air and water charged to

the vessel being the following:

(a) Asphalt charge stock, as gallons per minute, about 1;

65 (b) Air, as cubic feet per minute, about 10; and

(c) Water, as gallons per minute, up to about 0.05.

#### References Cited in the file of this patent

#### UNITED STATES PATENTS

|           |               |               |
|-----------|---------------|---------------|
| 1,988,766 | Aldridge      | Jan. 22, 1935 |
| 2,032,546 | McNeil et al. | Mar. 3, 1936  |
| 2,099,448 | McNeil et al. | Nov. 16, 1937 |
| 2,661,323 | Kraft         | Dec. 1, 1953  |